# EUROPEAN PATENT SPECIFICATION

(11) **EP 1 149 188 B1**
(45) Date of publication and mention of the grant of the patent: **11.09.2002**
(21) Application number: 00900036.5
(22) Date of filing: 10.01.2000
(51) Int. Cl.: C25C 3/12, C25C 7/02

(54) **HIGH-STRENGTH LOW-ALLOY STEEL ANODES FOR ALUMINIUM ELECTROWINNING CELLS**
ANODEN AUS HOCHFESTEM, NIEDRIGLEGIERTEM STAHL FÜR ZELLEN ZUR ALUMINIUM-SCHMELZELEKTROLYSE
ANODES EN ACIER HAUTE RESISTANCE FAIBLEMENT ALLIE POUR CELLULES D'EXTRACTION ELECTROLYTIQUE DE L'ALUMINIUM

(30) Priority: 08.01.1999 WO PCT/IB99/00015
(43) Date of publication of application: 31.10.2001
(73) Proprietor: MOLTECH Invent S.A., 2320 Luxembourg (LU)
(72) Inventor: DE NORA, Vittorio, Nassau (BS); DURUZ, Jean-Jacques, CH-1204 Geneva (CH)
(74) Representative: Cronin, Brian
(86) International application number: IB0000028
(87) International publication number: WO00040783

(56) References cited:
- US-A- 5 510 008

## Description

### Field of the Invention

This invention relates to non-carbon, metal-based, anodes for use in cells for the electrowinning of aluminium from alumina dissolved in a fluoride-containing molten electrolyte such as cryolite, and to methods for their fabrication, as well as to electrowinning cells containing such anodes and their use to produce aluminium.

### Background Art

The technology for the production of aluminium by the electrolysis of alumina, dissolved in molten cryolite, at temperatures around 950°C is more than one hundred years old.

This process conceived almost simultaneously by Hall and Héroult, has not evolved as many other electrochemical processes.

The anodes are still made of carbonaceous material and must be replaced every few weeks. During electrolysis the oxygen which should evolve on the anode surface combines with the carbon to form polluting CO₂ and small amounts of CO and fluorine-containing dangerous gases. The actual consumption of the anode is as much as 450 Kg/Ton of aluminium produced which is more than 1/3 higher than the theoretical amount of 333 Kg/Ton.

Using metal anodes in aluminium electrowinning cells would drastically improve the aluminium process by reducing pollution and the cost of aluminium production.

US Patent 4,999,097 (Sadoway) describes anodes for conventional aluminium electrowinning cells provided with an oxide coating containing at least one oxide of zirconium, hafnium, thorium and uranium. To prevent consumption of the anode, the bath is saturated with the materials that form the coating. However, these coatings are poorly conductive and have not been used.

US Patent 4,504,369 (Keller) discloses a method of producing aluminium in a conventional cell using anodes whose dissolution into the electrolytic bath is reduced by adding anode constituent materials into the electrolyte, allowing slow dissolution of the anode. However, this method is impractical because it would lead to a contamination of the product aluminium by the anode constituent materials which is considerably above the acceptable level in industrial production.

US Patent 4,614,569 (Duruz/Derivaz/Debely/Adorian) describes metal anodes for aluminium electrowinning coated with a protective coating of cerium oxyfluoride, formed in-situ in the cell or pre-applied, this coating being maintained during electrolysis by the addition of small amounts of a cerium compound to the molten cryolite electrolyte. This made it possible to have a protection of the surface from the electrolyte attack and to a certain extent from gaseous oxygen but not from nascent monoatomic oxygen.

EP Patent application 0 306 100 (Nyguen/Lazouni/Doan) describes anodes composed of a chromium, nickel, cobalt and/or iron based substrate covered with an oxygen barrier layer and a ceramic coating of nickel, copper and/or manganese oxide which may be further covered with an in-situ formed protective cerium oxyfluoride layer. Likewise, US Patents 5,069,771, 4,960,494 and 4,956,068 (all Nyguen/Lazouni/Doan) disclose aluminium production anodes with an oxidised copper-nickel surface on an alloy substrate with a protective barrier layer. However, full protection of the alloy substrate was difficult to achieve.

Metal or metal-based anodes are highly desirable in aluminium electrowinning cells instead of carbon-based anodes. Many attempts were made to use metallic anodes for aluminium production, however they were never adopted by the aluminium industry because they had a short life and contaminated the aluminium produced.

### Objects of the Invention

A major object of the invention is to provide an anode for aluminium electrowinning which has no carbon so as to eliminate carbon-generated pollution and increase the anode life.

A further object of the invention is to provide an aluminium electrowinning anode material with a surface having a high electrochemical activity and a low solubility in the electrolyte.

Another object of the invention is to provide an anode for the electrowinning of aluminium which is covered with an electrochemically active layer with limited ionic conductivity for oxygen ions.

Yet another object of the invention is to provide an anode for the electrowinning of aluminium which is made of readily available material(s).

An important object of the invention is to substantially reduce the solubility of the surface layer of an aluminium electrowinning anode, thereby maintaining the anode dimensionally stable.

Yet another object of the invention is to provide operating conditions for an aluminium electrowinning cell under which the contamination of the product aluminium is limited.

### Summary of the Invention

This invention is based on the observation that low-carbon high-strength low-alloy (HSLA) steels such as Cor-Ten™ even at high temperature form under oxidising conditions an iron oxide-based surface layer which is dense, electrically conductive, electrochemically active for oxygen evolution and, as opposed to oxide layers formed on standard steels or other iron alloys, is highly adherent and less exposed to delamination and limits diffusion of ionic, monoatomic and molecular oxygen.

HSLA steels are used for their strength and resistance to atmospheric corrosion especially at lower temperatures (below 0°C) in different areas of technology such as civil engineering (bridges, dock walls, sea walls, piping), architecture (buildings, frames) and mechanical engineering (welded/bolted/riveted structures, car and railway industry, high pressure vessels). However, these HSLA steels have never been proposed for applications at high temperature, especially under oxidising or corrosive conditions, in particular in cells for the electrowinning of aluminium.

It has been found that the iron oxide-based surface layer formed on the surface of a HSLA steel under oxidising conditions limits also at elevated temperatures the diffusion of oxygen oxidising the surface of the HSLA steel. Thus, diffusion of oxygen through the surface layer decreases with an increasing thickness thereof.

If the HSLA steel is exposed to an oxidising environment which maintains or preserves the surface layer, the iron oxide-based surface layer grows until its thickness constitutes a sufficient barrier to oxygen and then remains dimensionally stable. If the HSLA steel is exposed to an environment promoting dissolution or delamination of the surface layer, the rate of formation of the iron oxide-based surface layer (by oxidation of the surface of the HSLA steel) reaches the rate of dissolution or delamination of the surface layer after a transitional period during which the surface layer grows or decreases to reach an equilibrium thickness in the specific environment.

### Anodes and Manufacture

) The invention relates in particular to an anode of a cell for the electrowinning of aluminium from alumina dissolved in a fluoride-containing molten electrolyte. This anode comprises a low-carbon high-strength low-alloy (HSLA) steel body or layer whose surface is oxidised to form a coherent and adherent outer iron oxide-based layer the surface of which is electrochemically active for the evolution of oxygen. The iron oxide-based layer has a low solubility in the molten electrolyte. The thickness of the iron oxide-based layer is such as to reduce or prevent diffusion of oxygen from the electrochemically active surface into the steel body or layer during use.

During steady operation the reduced rate of diffusion through the oxide-based layer can be such that oxygen only diffuses into the steel body or layer in a controlled manner without significant increase of the thickness of the oxide-based layer.

High-strength low-alloy (HSLA) steel designates a group of low-carbon steels (typically up to 0.5 weight% carbon of the total) that contain small amounts of alloying elements. These steels have better mechanical properties and sometimes better corrosion resistance than carbon steels.

The surface of the high-strength low-alloy steel body or layer may be oxidised in an electrolytic cell or in an oxidising atmosphere, in particular a relatively pure oxygen atmosphere. For instance the surface of the high-strength low-alloy steel body or layer may be oxidised in a first electrolytic cell and then transferred to an aluminium production cell. In an electrolytic cell oxidation would typically last 5 to 15 hours at 800 to 1000°C. Oxidation may also take place in air or in oxygen for 5 to 25 hours at 750 to 1150°C before electrolysis.

In order to prevent thermal shocks causing mechanical stresses, a high-strength low-alloy steel body or layer may be tempered or annealed after pre-oxidation. Alternatively, the high-strength low-alloy steel body or layer may be maintained at elevated temperature after pre-oxidation until immersion into the molten electrolyte of an aluminium production cell.

The high-strength low-alloy steel body or layer may comprise 94 to 98 weight% iron and carbon, the remaining constituents being one or more further metals selected from chromium, copper, nickel, silicon, titanium, tantalum, tungsten, vanadium, zirconium, aluminium, molybdenum, manganese and niobium, and possibly small amounts of at least one additive selected from boron, sulfur, phosphorus and nitrogen.

In one embodiment, the anode comprises a layer of high-strength low-alloy steel on an oxidation resistant metallic core. The layer of high-strength low-alloy steel may be applied on the metallic core before or after formation of the outer iron oxide-based layer.

The metallic core is preferably electrically highly conductive and may be made of copper or a copper alloy. To enhance the mechanical properties, the metallic core may contain minor amounts of at least one oxide, such as alumina, hafnia, yttria and/or zirconia. Furthermore, to enhance oxidation resistance, the metallic core may be coated with at least one metal selected from nickel, chromium, cobalt, iron, aluminium, hafnium, manganese, molybdenum, niobium, silicon, tantalum, titanium, tungsten, vanadium, yttrium and zirconium, and alloys, intermetallic compounds and combinations thereof.

The metallic core may be coated with an oxygen barrier layer of chromium and/or niobium.

The layer of high-strength low-alloy steel may be plasma sprayed, arc sprayed, slurry-applied or electrodeposited onto the metallic core. Alternatively, to enhance adhesion, the high-strength low-alloy steel layer may be bonded to the metallic core through at least one intermediate layer, in particular a film of silver, typically 0.1 to 10 micron thick, which is in intimate and continuous contact with the metallic core and with the steel layer, and/or at least one layer of nickel and/or copper.

The invention also relates to a bipolar electrode of a cell for the electrowinning of aluminium from alumina dissolved in a fluoride-containing electrolyte, comprising on its anodic side an anode as described above.

The high strength low allow (HSLA) steel body can also be bonded or connected to an electrically conductive anode structure of special design as disclosed in WO-A-00/40781 and WO-A-00/40782 (both in the name of de Nora).

One aspect of the invention is an anode precursor comprising a low-carbon high-strength low-alloy (HSLA) steel body or layer and which can be converted into a fully manufactured anode as described above by oxidising the surface of the steel body or layer to form the coherent and adherent outer iron oxide-based layer.

Another aspect of the invention is a method of manufacturing an anode as described above comprising:
- providing a low-carbon high-strength low-alloy (HSLA) steel body or layer; and
- oxidising the surface of the high-strength low-alloy steel body or layer to form the coherent and adherent outer iron oxide-based layer the surface of which is electrochemically active for the evolution of oxygen.

### Cells and Aluminium Production

A further aspect of the invention is a cell for the electrowinning of aluminium from alumina dissolved in a fluoride-containing molten electrolyte comprising at least one anode having a low-carbon high-strength low-alloy (HSLA) steel body or layer and an electrochemically active outer iron oxide-based layer whose surface is electrochemically active, as described above.

During normal operation the electrochemically active layer of the or each anode may be progressively further formed by surface oxidation of the steel body or layer by controlled oxygen diffusion through the electrochemically active layer, and progressively dissolved into the electrolyte at the electrolyte/anode interface, the rate of formation of the outer iron oxide-based layer being substantially equal to its rate of dissolution into the electrolyte.

However, it has been observed that this type of anode may be maintained dimensionally stable under specific cell operating conditions.

In known processes, even the least soluble anode material releases excessive amounts of constituents into the bath, which leads to an excessive contamination of the product aluminium. For example, the concentration of nickel (a frequent component of proposed metal-based anodes) found in aluminium produced in small scale tests at conventional cell operating temperatures is typically comprised between 800 and 2000 ppm, i.e. 4 to 10 times the maximum acceptable level which is 200 ppm.

Iron oxides and in particular hematite (Fe₂O₃) have a higher solubility than nickel in molten electrolyte. However, in industrial production the contamination tolerance of the product aluminium by iron is also much higher (up to 2000 ppm) than for other metal impurities.

Solubility is an intrinsic property of anode materials and cannot be changed otherwise than by modifying the electrolyte composition and/or the operating temperature of a cell.

Small scale tests utilising a NiFe₂O₄/Cu cermet anode and operating under steady conditions were carried out to establish the concentration of iron in molten electrolyte and in the product aluminium under different operating conditions.

In the case of iron oxide, it has been found that lowering the temperature of the electrolyte deacreases considerably the solubility of iron species. This effect can surprisingly be exploited to produce a major impact on cell operation by limiting the contamination of the product aluminium by iron.

Thus, it has been found that when the operating temperature of the cell is reduced below the temperature of conventional cells (950-970°C) an anode covered with an outer layer of iron oxide can be made dimensionally stable by maintaining a concentration of iron species and alumina in the molten electrolyte sufficient to reduce or suppress the dissolution of the iron-oxide layer, the concentration of iron species being low enough not to exceed the commercial acceptable level of iron in the product aluminium.

The presence of dissolved alumina in the electrolyte at the anode surface has a limiting effect on the dissolution of iron from the anode into the electrolyte, which reduces the concentration of iron species necessary to substantially stop dissolution of iron from the anode.

Therefore, anodes according to the invention may be kept dimensionally stable by maintaining a sufficient amount of dissolved alumina and iron species in the electrolyte to reduce or prevent dissolution of the outer oxide layer.

The cell should be operated at a sufficiently low temperature to limit the solubility of iron species in the electrolyte, thereby limiting contamination of the product aluminium by constituents of the outer iron oxide-based layer of the anode(s) to a commercially acceptable level.

When the cell is operated with a fluoride-based melt the operating temperature of the electrolyte should be below 910°C, usually from 730 to 870°C.

The amount of iron species and alumina dissolved in the electrolyte preventing dissolution of the iron oxide-based outside surface layer of the or each anode should be such that the product aluminium is contaminated by no more than 2000 ppm iron, preferably by no more than 1000 ppm iron, and even more preferably by no more than 500 ppm iron.

Usually the iron species are intermittently fed into the electrolyte, for instance together with alumina, to maintain the amount of iron species in the electrolyte constant which, at the operating temperature, prevents the dissolution of the iron oxide-based outside surface layer of the anodes. However, the iron species can also be continuously fed, for instance by dissolving a sacrificial electrode which continuously feeds the iron species into the electrolyte.

The iron species may be fed in the form of iron metal and/or an iron compound, in particular iron oxide, iron fluoride, iron oxyfluoride and/or an iron-aluminium alloy.

Advantageously, the cell may comprise an aluminium-wettable cathode which can be a drained cathode on which aluminium is produced and from which it continuously drains, as described in US Patent 5,651,874 (de Nora/Sekhar) and 5,683,559 (de Nora).

Usually, the cell is in a monopolar, multi-monopolar or in a bipolar configuration. The bipolar cell comprises a terminal cathode facing a terminal anode and thereinbetween at least one bipolar electrode, the anode(s) described above forming the anodic side of the or each bipolar electrode and/or of the terminal anode.

In such a bipolar cell an electric current is passed from the surface of the terminal cathode to the surface of the terminal anode as ionic current in the electrolyte and as electronic current through the bipolar electrodes, thereby producing aluminium on each cathode surface and oxygen on each anode surface.

Preferably, the cell comprises means to improve the circulation of the electrolyte between the anodes and facing cathodes and/or means to facilitate dissolution of alumina in the electrolyte. Such means can for instance be provided by the geometry of the cell as described in co-pending application WO 99/41429 (de Nora/Duruz) or by periodically moving the anodes as described in co-pending application WO 99/41430 (Duruz/Bellò).

Yet another aspect of the invention is a method of producing aluminium in a cell as described above. The method comprises dissolving alumina in the electrolyte and passing an ionic electric current between the electrochemically active surface of the anode(s) and the surface of the cathode(s), thereby producing aluminium on the cathode surface(s) and oxygen on the anode surface(s).

Yet a further aspect of the invention is a method of manufacturing an anode and producing aluminium in an electrolytic cell comprising inserting an anode precursor as described above into the electrolyte of an electrolytic cell and forming the iron oxide-based layer to produce a fully manufactured anode, and producing oxygen on the surface of the iron oxide-based layer and aluminium on a facing cathode in the same (or nearly the same) or in a different electrolyte.

The thus-produced anode may then be transferred from the electrolytic cell in which it was produced to an aluminium electrowinning cell. Alternatively the composition of the electrolyte in which the anode was produced can be suitably modified, for instance by dissolving alumina and optionally iron species, and electrolysis continued in the same cell to produce aluminium.

### Detailed Description

The invention will be further described in the following Examples:

### Example 1

Electrolysis was carried out in a laboratory scale cell equipped with an anode according to the invention.

The anode was made with a Cor-Ten™ type low-carbon high-strength (HSLA) steel containing niobium, titanium, chromium and copper in a total amount of less than 4 weight%. The anode was pre-oxidised in air at about 1050°C for 15 hours for the formation of a dense hematite-based outer layer.

The anode was then tested in a fluoride-containing molten electrolyte at 850°C and at a current density of about 0.7 A/cm². The electrolyte contained cryolite and 15 weight% excess of AlF₃, approximately 3 weight% alumina and approximately 200 ppm iron species obtained from the dissolution of iron oxide thereby surely saturating the electrolyte with iron species and inhibiting dissolution of the hematite-based anode surface layer.

To maintain the concentration of dissolved alumina in the electrolyte, fresh alumina was periodically fed into the cell. The alumina feed contained sufficient iron oxide so as to replace the iron which had been deposited into the product aluminium, thereby maintaining the concentration of iron in the electrolyte at the limit of solubility and preventing dissolution of the hematite-based anode surface layer.

After 140 hours electrolysis was interrupted and the anode extracted. Upon cooling the anode was examined externally and in cross-section. No corrosion was observed at or near the surface of the anode.

The produced aluminium was also analysed and showed an iron contamination of about 700 ppm which is below the tolerated iron contamination in commercial aluminium production.

### Example 2

As in Example 1, aluminium was produced in a laboratory scale cell equipped with an anode according to the invention.

The anode was made with a low-carbon high-strength (HSLA) steel containing manganese 0.4 weight%, niobium 0.02 weight%, molybdenum 0.02 weight%, copper 0.3 weight%, nickel 0.45 weight% and chromium 0.8 weight%. The anode was pre-oxidised in air at about 850°C for 12 hours to form a dense hematite-based outer layer.

The anode was then tested under similar conditions as in Example 1 and the test results were similar.

### Example 3

As in Example 1, aluminium was produced in a laboratory scale cell equipped with an anode according to the invention.

The anode was made with a low-carbon high-strength (HSLA) steel containing nickel, copper and silicon in a total amount of less than 1.5 weight%. The anode was pre-oxidised in air at about 850°C for 12 hours to form a dense hematite-based outer layer.

The anode was then tested under similar conditions as in Example 1 and the test results were similar.

## Claims

1. An anode of a cell for the electrowinning of aluminium from alumina dissolved in a fluoride-containing molten electrolyte, said anode comprising a low-carbon high-strength low-alloy (HSLA) steel body or layer whose surface is oxidised to form a coherent and adherent outer iron oxide-based layer the surface of which is electrochemically active for the evolution of oxygen, said iron oxide-based layer having a low solubility in the molten electrolyte, the thickness of said iron oxide-based layer being such as to reduce or prevent diffusion of oxygen from the electrochemically active surface into the steel body or layer.

2. The anode of claim 1, wherein the high-strength low-alloy steel body or layer comprises 94 to 98 weight% iron and carbon, the remaining constituents being one or more further metals selected from chromium, copper, nickel, silicon, titanium, tantalum, tungsten, vanadium, zirconium, aluminium, molybdenum, manganese and niobium, and possibly small amounts of at least one additive selected from boron, sulfur, phosphorus and nitrogen.

3. The anode of claim 1, comprising a layer of high-strength low-alloy steel on an oxidation resistant metallic core.

4. The anode of claim 3, wherein the metallic core is made of copper or a copper alloy, possibly containing minor amounts of at least one oxide reinforcing the mechanical properties of the metallic core.

5. The anode of claim 4, wherein said at least one reinforcing oxide is selected from alumina, hafnia, yttria and zirconia.

6. The anode of claim 3, wherein the metallic core is coated with at least one metal selected from nickel, chromium, cobalt, iron, aluminium, hafnium, manganese, molybdenum, niobium, silicon, tantalum, titanium, tungsten, vanadium, yttrium and zirconium, and alloys, intermetallic compounds and combinations thereof.

7. The anode of claim 6, wherein the metallic core is coated with an oxygen barrier layer of chromium and/or niobium.

8. The anode of claim 3, wherein the high-strength low-alloy steel layer is bonded to the metallic core through at least one intermediate layer.

9. The anode of claim 8, wherein the high-strength low-alloy steel layer is bonded to the metallic core through a film of silver, and/or at least one layer of nickel and/or copper.

10. A bipolar electrode of a cell for the electrowinning of aluminium from alumina dissolved in a fluoride-containing electrolyte, comprising on its anodic side an anode as defined in claim 1.

11. A method of manufacturing an anode as defined in claim 1 comprising:
- providing a low-carbon high-strength low-alloy (HSLA) steel body or layer; and
- oxidising the surface of the high-strength low-alloy steel body or layer to form the coherent and adherent outer iron oxide-based layer the surface of which is electrochemically active for the evolution of oxygen.

12. The method of claim 11, comprising applying a layer of high-strength low-alloy steel on an oxidation resistant metallic core before or after formation of said outer iron oxide-based layer.

13. The method of claim 12, comprising plasma spraying, arc spraying or electrodepositing the high-strength low-alloy steel layer on the metallic core.

14. The method of claim 12, comprising bonding the high-strength low-alloy steel layer to the metallic core through at least one intermediate bonding layer.

15. The method of claim 11, comprising oxidising the surface of the high-strength low-alloy steel body or layer in a molten electrolyte at 800 to 1000°C for 5 to 15 hours.

16. The method of claim 15, comprising oxidising the surface of the high-strength low-alloy steel body or layer at 750 to 1150°C for 5 to 25 hours in an oxidising atmosphere such as air or oxygen before electrolysis.

17. A cell for the electrowinning of aluminium from alumina dissolved in a fluoride-containing molten electrolyte comprising at least one anode having a low-carbon high-strength low-alloy (HSLA) steel body or layer and an electrochemically active outer iron oxide-based layer as defined in claim 1.

18. The cell of claim 17, wherein during normal operation the electrochemically active layer of the or each anode is progressively further formed by surface oxidation of the steel body or layer by controlled oxygen diffusion through the electrochemically active layer, and progressively dissolved into the electrolyte at the electrolyte/anode interface, the rate of formation of the outer iron oxide-based layer being substantially equal to its rate of dissolution into the electrolyte.

19. The cell of claim 17, wherein the or each anode is kept dimensionally stable by maintaining a sufficient amount of dissolved alumina and iron species in the electrolyte to prevent dissolution of the outer oxide layer of the or each anode.

20. The cell of claim 19, which is operated at a sufficiently low temperature to limit the solubility of the outer iron oxide-based layer of the anode(s), thereby limiting the contamination of the product aluminium by constituents of the outer iron oxide-based layer of the anode(s).

21. The cell of claim 17, which is in a bipolar configuration, comprising a terminal cathode facing a terminal anode and thereinbetween at least one bipolar electrode, and wherein said anode(s) form(s) the anodic side of the or each bipolar electrode and/or the terminal anode.

22. A method of producing aluminium in a cell as defined in claim 17, the method comprising dissolving alumina in the electrolyte and passing an ionic electric current between the electrochemically active surface of the anode(s) and the surface of the cathode(s), thereby producing aluminium on the cathode surface(s) and oxygen on the anode surface(s).

23. The method of claim 22, wherein the electrochemically active layer of the or each anode is progressively further formed by surface oxidation of the steel body or layer by controlled oxygen diffusion through the electrochemically layer, and progressively dissolved into the electrolyte at the electrolyte/anode interface, the rate of formation of the outer iron oxide-based layer being substantially equal to its rate of dissolution into the electrolyte.

24. The method of claim 22, comprising keeping the or each anode dimensionally stable by maintaining a sufficient amount of dissolved alumina and iron species in the electrolyte to prevent dissolution of the outer oxide layer of the or each anode.

25. The method of claim 22, comprising operating the cell at a sufficiently low temperature to limit the solubility of the outer iron oxide-based layer of the anode(s), thereby limiting contamination of the product aluminium by constituents of the outer iron oxide-based layer of the anode(s).

26. The method of claim 25, wherein the cell is operated with an operative temperature of the electrolyte below 910°C.

27. The method of claim 26, wherein the cell is operated at an electrolyte temperature from 730 to 870°C.

28. The method of claim 25, wherein the amount of iron species and alumina dissolved in the electrolyte preventing dissolution of the iron oxide-based outside surface layer of the or each anode is such that the product aluminium is contaminated by no more than 2000 ppm iron, preferably by no more than 1000 ppm iron, and even more preferably by no more than 500 ppm iron.

29. The method of claim 24, wherein iron species are intermittently or continuously fed into the electrolyte to maintain the amount of iron species in the electrolyte which prevents at the operating temperature the dissolution of the iron oxide-based outside surface layer of the or each anode.

30. The method of claim 29, wherein the iron species are fed in the form of iron metal and/or an iron compound.

31. The method of claim 30, wherein the iron species are fed into the electrolyte in the form of iron oxide, iron fluoride, iron oxyfluoride and/or an iron-aluminium alloy.

32. The method of claim 29, wherein the iron species are periodically fed into the electrolyte together with alumina.

33. The method of claim 29, wherein a sacrificial electrode continuously feeds the iron species into the electrolyte.

34. The method of claim 22, for producing aluminium on an aluminium-wettable cathode.

35. The method of claim 34, wherein the produced aluminium continuously drains from said cathode.

36. The method of claim 22, comprising circulating the electrolyte between the anodes and facing cathodes thereby improving dissolution of alumina into the electrolyte and/or improving the supply of dissolved alumina under the active surfaces of the anodes.

37. Use of a low-carbon high-strength low-alloy (HSLA) steel body or layer as an anode precursor which can be converted into an aluminium electrowinning anode as defined in claim 1 by oxidising the surface of the steel body or layer to form the coherent and adherent outer iron oxide-based layer.

38. A method of manufacturing an anode and producing aluminium in an electrolytic cell comprising inserting a low-carbon high-strength low-alloy (HSLA) steel body or layer as an anode precursor into a fluoride-containing molten electrolyte of an electrolytic cell, oxidising in-situ the surface of the anode precursor to produce an electrochemically active iron oxide-based layer, thereby converting the anode precursor into an anode as defined in claim 1, and producing oxygen on the surface of the iron oxide-based layer and aluminium on a facing cathode in the same or in a different electrolyte.

## Patentansprüche

1. Anode von einer Zelle für die elektrolytische Gewinnung von Aluminium aus Aluminiumoxid, das in einem fluoridhaltigen, geschmolzenen Elektrolyten gelöst ist, wobei die Anode einen Körper oder eine Schicht aus einem kohlenstoffarmen, hochfesten, niedriglegierten (HSLA)-Stahl aufweist, deren Oberfläche oxidiert ist, um eine kohärente und haftende äußere, auf Eisenoxid basierende Schicht zu bilden, deren Oberfläche für die Sauerstoffentwicklung elektrochemisch aktiv ist, wobei die auf Eisenoxid basierende Schicht eine geringe Löslichkeit in dem geschmolzenen Elektrolyten besitzt und die Dicke der auf Eisenoxid basierenden Schicht so ist, dass die Diffusion von Sauerstoff von der elektrochemisch aktiven Oberfläche in den Stahlkörper oder die Stahlschicht vermindert oder verhindert wird.

2. Anode nach Anspruch 1, bei der der Körper oder die Schicht aus hochfestem, niedriglegierten Stahl 94-98 Gew.-% Eisen und Kohlenstoff enthält, wobei die übrigen Bestandteile ein oder mehrere weitere Metalle, die aus Chrom, Kupfer, Nickel, Silizium, Titan, Tantal, Wolfram, Vanadium, Zirkonium, Aluminium, Molybdän, Mangan und Niob ausgewählt sind, sowie gegebenenfalls geringe Mengen von mindestens einem Additiv sind, das aus Bor, Schwefel, Phosphor und Stickstoff ausgewählt ist.

3. Anode nach Anspruch 1, mit einer Schicht aus hochfestem, niedriglegierten Stahl auf einem oxidationsbeständigen metallischen Kern.

4. Anode nach Anspruch 3, bei der der metallische Kern aus Kupfer oder einer Kupferlegierung hergestellt ist und gegebenenfalls geringe Mengen von mindestens einem Oxid enthält, wodurch die mechanischen Eigenschaften des metallischen Kerns verstärkt werden.

5. Anode nach Anspruch 4, bei der das mindestens eine verstärkende Oxid aus Aluminiumoxid, Hafniumoxid, Yttriumoxid und Zirkonoxid ausgewählt ist.

6. Anode nach Anspruch 3, bei der der metallische Kern mit mindestens einem Metall beschichtet ist, das ausgewählt ist aus Nickel, Chrom, Kobalt, Eisen, Aluminium, Hafnium, Mangan, Molybdän, Niob, Silizium, Tantal, Titan, Wolfram, Vanadium, Yttrium und Zirkonium, sowie Legierungen, intermetallischen Verbindungen und Kombinationen derselben.

7. Anode nach Anspruch 6, bei der der metallische Kern mit einer Sauerstoffsperrschicht aus Chrom und/oder Niob beschichtet ist.

8. Anode nach Anspruch 3, bei der die Schicht aus hochfestem, niedriglegierten Stahl auf dem metallischen Kern durch mindestens eine Zwischenschicht gebunden ist.

9. Anode nach Anspruch 8, bei der die Schicht aus hochfestem, niedriglegierten Stahl auf dem metallischen Kern durch einen Film aus Silber und/oder mindestens eine Schicht aus Nickel und/oder Kupfer gebunden ist.

10. Bipolare Elektrode von einer Zelle für die elektrolytische Gewinnung von Aluminium aus Aluminiumoxid, das in einem fluoridhaltigen Elektrolyten gelöst ist, mit einer Anode gemäß Anspruch 1 an ihrer anodischen Seite.

11. Verfahren zur Herstellung einer Anode gemäß Anspruch 1, mit:
Bereitstellen eines Körpers oder einer Schicht aus einem kohlenstoffarmen, hochfesten, niedriglegierten (HSLA)-Stahl; und
Oxidieren der Oberfläche des Körpers oder der Schicht aus hochfestem, niedriglegierten Stahl, um die kohärente und haftende äußere, auf Eisenoxid basierende Schicht zu bilden, deren Oberfläche für de Sauerstoffentwicklung elektrochemisch aktiv ist.

12. Verfahren nach Anspruch 11, mit dem Aufbringen einer Schicht aus hochfestem, niedriglegierten Stahl auf einen oxidationsbeständigen, metallischen vor oder nach Bildung der äußeren, auf Eisenoxid basierenden Schicht.

13. Verfahren nach Anspruch 12, bei dem die Schicht aus hochfestem, niedriglegierten Stahl auf den metallischen Kern plasmagesprüht, im Lichtbogen gesprüht oder elektrolytisch abgeschieden wird.

14. Verfahren nach Anspruch 12, bei dem die Schicht aus hochfestem, niedriglegierten Stahl durch mindestens eine Zwischenbindungsschicht auf den metallischen Kern gebunden wird.

15. Verfahren nach Anspruch 11, bei dem die Oberfläche des Körpers oder der Schicht aus hochfestem, niedriglegierten Stahl in einem geschmolzenen Elektrolyten 5 bis 15 Stunden lang bei 800°C bis 1000°C oxidiert wird.

16. Verfahren nach Anspruch 15, bei dem die Oberfläche des Körpers oder der Schicht aus hochfestem, niedriglegierten Stahl vor der Elektrolyse 5 bis 25 Stunden lang bei 750°C bis 1150°C in einer oxidierenden Atmosphäre, wie Luft oder Sauerstoff, oxidiert wird.

17. Zelle für die elektrolytische Gewinnung von Aluminium aus Aluminiumoxid, das in einem fluoridhaltigen, geschmolzenen Elektrolyten gelöst ist, mit mindestens einer Anode mit einem Körper oder einer Schicht aus einem kohlenstoffarmen, hochfesten, niedriglegierten (HSLA)-Stahl und einer elektrochemisch aktiven, äußeren, auf Eisenoxid basierenden Schicht gemäß Anspruch 1.

18. Zelle nach Anspruch 17, bei der beim normalem Betrieb die elektrochemisch aktive Schicht der oder jeder Anode durch Oberflächenoxidation des Stahlkörpers oder der Stahlschicht durch kontrollierte Sauerstoffdiffusion durch die elektrochemisch aktive Schicht fortschreitend weiter gebildet wird und an der Elektrolyt/Anoden-Grenzfläche fortschreitend in den Elektrolyten aufgelöst wird, wobei die Bildungsgeschwindigkeit der äußeren, auf Eisenoxid basierenden Schicht im wesentlichen gleich ihrer Auflösungsgeschwindigkeit in den Elektrolyten ist.

19. Zelle nach Anspruch 17, bei der die oder jede Anode dimensionsstabil gehalten wird, indem eine ausreichende Menge von gelöstem Aluminiumoxid und Eisenspezies in dem Elektrolyten aufrechterhalten wird, um eine Auflösung der äußeren Oxidschicht der oder jeder Anode zu verhindern.

20. Zelle nach Anspruch 19, die bei einer ausreichend niedrigen Temperatur betrieben wird, um die Löslichkeit der äußeren, auf Eisenoxid basierenden Schicht der Anode(n) zu begrenzen, wodurch die Verunreinigung des Produkt-Aluminiums durch Bestandteile der äußeren, auf Eisenoxid basierenden Schicht der Anode(n) begrenzt wird.

21. Zelle nach Anspruch 17, die in einer bipolaren Anordnung geschaltet ist, mit einer Anschluß-Kathode, die einer Anschluß-Anode gegenüberliegt, und dazwischen mit mindestens einer bipolaren Elektrode, wobei die Anode(n) die anodische Seite der oder jeder bipolaren Elektrode und/oder der Anschluß-Anode bildet (bilden).

22. Verfahren zur Herstellung von Aluminium in einer Zelle gemäß Anspruch 17, wobei das Verfahren umfasst: Lösen von Aluminiumoxid in dem Elektrolyten und Leiten von einem ionischen, elektrischen Strom zwischen der elektrochemisch aktiven Oberfläche der Anode(n) und der Oberfläche der Kathode(n), wodurch Aluminium an der Kathodenoberfläche(n) und Sauerstoff an der Anodenoberfläche(n) hergestellt wird.

23. Verfahren nach Anspruch 22, bei dem die elektrochemisch aktive Schicht der oder jeder Anode durch Oberflächenoxidation des Stahlkörpers oder der Stahlschicht durch kontrollierte Sauerstoffdiffusion durch die elektrochemisch aktive Schicht fortschreitend weiter gebildet wird und an der Elektrolyt/Anoden-Grenzfläche fortschreitend in den Elektrolyten aufgelöst wird, wobei die Bildungsgeschwindigkeit der äußeren, auf Eisenoxid basierenden Schicht im wesentlichen gleich ihrer Auflösungsgeschwindigkeit in den Elektrolyten ist.

24. Verfahren nach Anspruch 22, bei dem die oder jede Anode dimensionsstabil gehalten wird, indem eine ausreichende Menge von gelöstem Aluminiumoxid und Eisenspezies in dem Elektrolyten aufrechterhalten wird, um eine Auflösung der äußeren Oxidschicht der oder jeder Anode zu verhindern.

25. Verfahren nach Anspruch 22, bei dem die Zelle bei einer ausreichend niedrigen Temperatur betrieben wird, um die Löslichkeit der äußeren, auf Eisenoxid basierenden Schicht der Anode(n) zu begrenzen, wodurch die Verunreinigung des Produkt-Aluminiums durch Bestandteile der äußeren, auf Eisenoxid basierenden Schicht der Anode(n) begrenzt wird.

26. Verfahren nach Anspruch 25, bei dem die Zelle mit einer Betriebstemperatur des Elektrolyten unter 910°C betrieben wird.

27. Verfahren nach Anspruch 26, bei dem die Zelle bei einer Elektrolyt-Temperatur von 730°C bis 870°C betrieben wird.

28. Verfahren nach Anspruch 25, bei dem die Menge von Eisenspezies und Aluminiumoxid, die in dem Elektrolyten aufgelöst sind, wodurch die Auflösung der auf Eisenoxid basierenden, äußeren Oberflächenschicht der oder jeder Anode verhindert wird, so ist, dass das Produkt-Aluminium mit nicht mehr als 2000 ppm Eisen, vorzugsweise nicht mehr als 1000 ppm Eisen und insbesondere nicht mehr als 500 ppm Eisen, verunreinigt ist.

29. Verfahren nach Anspruch 24, bei dem Eisenspezies diskontinuierlich oder kontinuierlich in den Elektrolyten eingebracht werden, um die Menge von Eisenspezies in dem Elektrolyten aufrechtzuerhalten, die bei der Betriebstemperatur die Auflösung der auf Eisenoxid basierenden, äußeren Oberflächenschicht der oder jeder Anode verhindert.

30. Verfahren nach Anspruch 29, bei dem die Eisenspezies in Form von metallischem Eisen und/oder Eisenverbindung eingebracht werden.

31. Verfahren nach Anspruch 30, bei dem die Eisenspezies in den Elektrolyten in Form von Eisenoxid, Eisenfluorid, Eisenoxyfluorid und/oder Eisen-Aluminium-Legierung eingebracht werden.

32. Verfahren nach Anspruch 29, bei dem die Eisenspezies periodisch zusammen mit Aluminiumoxid in den Elektrolyten eingebracht werden.

33. Verfahren nach Anspruch 29, bei dem eine Opferelektrode die Eisenspezies kontinuierlich in den Elektrolyten einbringt.

34. Verfahren nach Anspruch 22 zur Herstellung von Aluminium auf einer mit Aluminium benetzbaren Kathode.

35. Verfahren nach Anspruch 34, bei dem das hergestellte Aluminium kontinuierlich von der Kathode abläuft.

36. Verfahren nach Anspruch 22, bei dem der Elektrolyt zwischen den Anoden und gegenüberliegenden Kathoden zirkuliert wird, wodurch die Auflösung von Aluminiumoxid in den Elektrolyten verbessert und/oder die Zufuhr von gelöstem Aluminiumoxid unter die aktiven Oberflächen der Anoden verbessert wird.

37. Verwendung eines Körpers oder einer Schicht aus kohlenstoffarmem, hochfesten, niedriglegierten (HSLA)-Stahl als Anoden-Vorläufer, der durch Oxidieren der Oberfläche des Stahlkörpers oder der Stahlschicht in eine Anode für die elektrolytischen Gewinnung von Aluminium gemäß Anspruch 1 umgewandelt werden kann, um die kohärente und haftende, äußere, auf Eisenoxid basierende Schicht zu bilden.

38. Verfahren zur Herstellung einer Anode und zur Produktion von Aluminium in einer Elektrolysezelle, mit dem Einsetzen eines Körper oder einer Schicht aus einem kohlenstoffarmen, hochfesten, niedriglegierten (HSLA)-Stahl als ein Anoden-Vorläufer in einen fluoridhaltigen, geschmolzenen Elektrolyten von einer Elektrolysezelle, Oxidieren der Oberfläche des Anoden-Vorläufers in-situ, um eine elektrochemisch aktive, auf Eisenoxid basierende Schicht herzustellen, wodurch den Anoden-Vorläufer in eine Anode nach Anspruch 1 umgewandelt wird, und Erzeugen von Sauerstoff an der Oberfläche der auf Eisenoxid basierenden Schicht und Aluminium an einer gegenüberliegenden Kathode in dem gleichen oder in einem unterschiedlichen Elektrolyten.

## Revendications

1. Anode d'une cuve pour l'électro-obtention d'aluminium à partir d'alumine dissoute dans un électrolyte fondu contenant du fluorure, ladite anode comprenant une couche ou un corps d'acier faiblement allié à haute résistance (HSLA) à faible teneur en carbone, dont la surface est oxydée pour former une couche à base d'oxyde de fer externe, cohérente et adhérente, dont la surface est électrochimiquement active pour le dégagement d'oxygène, ladite couche à base d'oxyde de fer ayant une faible solubilité dans l'électrolyte fondu, l'épaisseur de ladite couche à base d'oxyde de fer étant telle qu'elle réduit ou empêche la diffusion d'oxygène à partir de la surface électrochimiquement active dans le corps ou la couche d'acier.

2. Anode selon la revendication 1, dans laquelle le corps ou la couche d'acier faiblement allié à haute résistance comprend 94 à 98% en poids de fer et de carbone, les constituants restants étant l'un ou plusieurs des autres métaux choisis à partir du chrome, cuivre, nickel, silicium, titane, tantale, tungstène, vanadium, zirconium, aluminium, molybdène, manganèse et niobium et, éventuellement, de petites quantités d'au moins un additif choisi à partir du bore, soufre, phosphore et azote.

3. Anode selon la revendication 1, comprenant une couche d'acier faiblement allié à haute résistance sur un noyau métallique résistant à l'oxydation.

4. Anode selon la revendication 3, dans laquelle le noyau métallique est réalisé en cuivre ou en alliage de cuivre, contenant éventuellement des quantités mineures d'au moins un oxyde renforçant les propriétés mécaniques du noyau métallique.

5. Anode selon la revendication 4, dans laquelle ledit oxyde de renfort est choisi à partir d'alumine, d'oxyde de hafnium, d'yttria et de zircone.

6. Anode selon la revendication 3, dans laquelle le noyau métallique est revêtu d'au moins un métal choisi à partir de nickel, chrome, cobalt, fer, aluminium, hafnium, manganèse, molybdène, niobium, silicium, tantale, titane, tungstène, vanadium, yttrium et zirconium, et des alliages, composés intermétalliques et combinaisons de ceux-ci.

7. Anode selon la revendication 6, dans laquelle le noyau métallique est enrobé d'une couche d'arrêt à l'oxygène de chrome et/ou de niobium.

8. Anode selon la revendication 3, dans laquelle la couche d'acier faiblement allié à haute résistance est liée au noyau métallique par au moins une couche intermédiaire.

9. Anode selon la revendication 8, dans laquelle la couche d'acier faiblement allié à haute résistance est liée au noyau métallique par un film d'argent, et/ou au moins une couche de nickel et/ou de cuivre.

10. Electrode bipolaire d'une cuve pour l'électro-obtention d'aluminium à partir d'alumine dissoute dans un électrolyte contenant du fluorure, comprenant sur son côté anodique une anode telle que définie dans la revendication 1.

11. Procédé de fabrication d'une anode telle que définie dans la revendication 1 consistant à :
- fournir un corps ou une couche d'acier faiblement allié à haute résistance (HSLA) à faible teneur en carbone ; et
- oxyder la surface du corps ou de la couche d'acier faiblement allié à haute résistance pour former la couche à base d'oxyde de fer externe cohérente et adhérente, dont la surface est électrochimiquement active pour le dégagement d'oxygène.

12. Procédé selon la revendication 11, consistant à appliquer une couche d'acier faiblement allié à haute résistance sur un noyau métallique résistant à l'oxydation avant ou après la formation de ladite couche à base d'oxyde de fer externe.

13. Procédé selon la revendication 12, consistant à effectuer une projection au plasma, une projection à l'arc ou un dépôt par électrolyse de la couche d'acier faiblement allié à haute résistance sur le noyau métallique.

14. Procédé selon la revendication 12, consistant à lier la couche d'acier faiblement allié à haute résistance au noyau métallique via au moins une couche de liaison intermédiaire.

15. Procédé selon la revendication 11, consistant à oxyder la surface du corps ou de la couche d'acier faiblement allié à haute résistance dans un électrolyte fondu à 800 à 1000°C pendant 5 à 15 heures.

16. Procédé selon la revendication 15, consistant à oxyder la surface du corps ou de la couche d'acier faiblement allié à haute résistance à 750 à 1150°C pendant 5 à 25 heures dans une atmosphère oxydante telle que de l'air ou de l'oxygène avant électrolyse.

17. Cuve pour l'électro-obtention d'aluminium à partir d'alumine dissoute dans un électrolyte fondu contenant du fluorure, comprenant au moins une anode ayant un corps ou une couche d'acier faiblement allié à haute résistance (HSLA) à faible teneur en carbone et une couche à base d'oxyde de fer externe, électrochimiquement active, telle que définie dans la revendication 1.

18. Cuve selon la revendication 17, dans laquelle, pendant le fonctionnement normal, la couche électrochimiquement active de l'anode ou de chaque cathode est progressivement formée encore par oxydation de surface du corps ou de la couche d'acier par diffusion d'oxygène contrôlée via la couche électrochimiquement active, et progressivement dissoute dans l'électrolyte au niveau de l'interface électrolyte/anode, la vitesse de formation de la couche à base d'oxyde de fer externe étant sensiblement égale à sa vitesse de dissolution dans l'électrolyte.

19. Cuve selon la revendication 17, dans laquelle l'anode ou chaque anode est conservée dimensionnellement stable en maintenant une quantité suffisante d'alumine dissoute et d'espèces de fer dans l'électrolyte pour empêcher la dissolution de la couche d'oxyde externe de l'anode ou de chaque anode.

20. Cuve selon la revendication 19, qui fonctionne à une température suffisamment basse pour limiter la solubilité de la couche à base d'oxyde de fer, externe, de l'anode(s), en limitant ainsi la contamination de l'aluminium produit par des constituants de la couche à base d'oxyde de fer externe de l'anode(s).

21. Cuve selon la revendication 17, qui est dans une configuration bipolaire, comprenant une cathode de borne faisant face à une anode de borne et entre elles au moins une électrode bipolaire, et dans laquelle ladite anode(s) forme(nt) le côté anodique de l'électrode bipolaire ou de chaque électrode bipolaire et/ou l'anode de borne.

22. Procédé pour produire de l'aluminium dans une cuve comme défini dans la revendication 17, le procédé consistant à dissoudre de l'alumine dans l'électrolyte et à faire passer un courant électrique ionique entre la surface électrochimiquement active de l'anode(s) et la surface de la cathode(s), en produisant ainsi de l'aluminium sur la surface(s) de cathode et l'oxygène sur la surface(s) d'anode.

23. Procédé selon la revendication 22, dans lequel la couche électrochimiquement active de l'anode ou de chaque anode est progressivement formée de plus par oxydation de surface du corps ou de la couche d'acier par diffusion d'oxygène contrôlée à travers la couche électrochimiquement active, et est progressivement dissoute dans l'électrolyte au niveau de l'interface électrolyte/anode, la vitesse de formation de la couche externe à base d'oxyde de fer étant sensiblement égale à sa vitesse de dissolution dans l'électrolyte.

24. Procédé selon la revendication 22, consistant à conserver l'anode ou chaque anode dimensionnellement stable en maintenant une quantité suffisante d'alumine dissoute et d'espèces de fer dans l'électrolyte pour empêcher la dissolution de la couche d'oxyde externe de l'anode ou de chaque anode.

25. Procédé selon la revendication 22, consistant à faire fonctionner la cuve à une température suffisamment basse pour limiter la solubilité de la couche externe à base d'oxyde de fer de l'anode(s), en limitant ainsi la contamination de l'aluminium produit par des constituants de la couche externe à base d'oxyde de fer de l'anode(s).

26. Procédé selon la revendication 25, dans lequel la cuve fonctionne à une température opératoire de l'électrolyte en dessous de 910°C.

27. Procédé selon la revendication 26, dans lequel la cuve fonctionne à une température d'électrolyte de 730 à 870°C.

28. Procédé selon la revendication 25, dans lequel la quantité d'espèces de fer et d'alumine dissoute dans l'électrolyte empêchant la dissolution de la couche de surface extérieure à base d'oxyde de fer de l'anode ou de chaque anode, est telle que l'aluminium produit est contaminé par pas plus de 2000 ppm de fer, de préférence, par pas plus de 1000 ppm de fer, et même plus préférablement par pas plus de 500 ppm de fer.

29. Procédé selon la revendication 24, dans lequel des espèces de fer sont fournies de façon intermittente ou continue dans l'électrolyte pour maintenir la quantité d'espèces de fer dans l'électrolyte qui empêche, à la température de fonctionnement, la dissolution de la couche de surface extérieure à base d'oxyde de fer de l'anode ou de chaque anode.

30. Procédé selon la revendication 29, dans lequel les espèces de fer sont fournies sous la forme de métal de fer et/ou d'un composé de fer.

31. Procédé selon la revendication 30, dans lequel les espèces de fer sont fournies dans l'électrolyte sous la forme d'oxyde de fer, de fluorure de fer, d'oxyfluorure de fer et/ou d'un alliage fer-aluminium.

32. Procédé selon la revendication 29, dans lequel les espèces de fer sont périodiquement fournies dans l'électrolyte en même temps que l'alumine.

33. Procédé selon la revendication 29, dans lequel une électrode soluble fournit de façon continue les espèces de fer dans l'électrolyte.

34. Procédé selon la revendication 22, pour produire de l'aluminium sur une cathode mouillable par l'aluminium.

35. Procédé selon la revendication 34, dans lequel l'aluminium produit est drainé de façon continue à partir de ladite cathode.

36. Procédé selon la revendication 22, consistant à mettre en circulation l'électrolyte entre les anodes et cathodes en vis-à-vis en améliorant ainsi la dissolution d'alumine dans l'électrolyte et/ou en améliorant l'amenée d'alumine dissoute sous les surfaces actives des anodes.

37. Utilisation d'un corps ou d'une couche d'acier faiblement allié à haute résistance (HSLA) à faible teneur en carbone, comme un précurseur d'anode qui peut être transformé en une anode d'électro-obtention d'aluminium telle que définie dans la revendication 1 par oxydation de la surface du corps ou de la couche d'acier pour former la couche externe à base de fer, cohérente et adhérente.

38. Procédé pour fabriquer une anode et produire de l'aluminium dans une cuve électrolytique consistant à insérer un corps ou une couche d'acier faiblement allié à haute résistance (HSLA) à faible teneur en carbone comme un précurseur d'anode dans un électrolyte fondu contenant du fluorure d'une cuve électrolytique, à oxyder in situ la surface du précurseur d'anode pour produire une couche à base d'oxyde de fer électrochimiquement active, en transformant ainsi le précurseur d'anode en une anode telle que définie dans la revendication 1, et à produire de l'oxygène sur la surface de la couche à base d'oxyde de fer et de l'aluminium sur une cathode faisant face dans le même électrolyte ou dans un électrolyte différent.
